

# UNITED STATES PATENT OFFICE.

WILHELM LESSING, OF TROISDORF, GERMANY.

## ORE-BRIQUETING.

952,914.

Specification of Letters Patent. Patented Mar. 22, 1910.

No Drawing.

Application filed August 14, 1908. Serial No. 448,544.

To all whom it may concern:

Be it known that I, WILHELM LESSING, a subject of the German Emperor, residing at Troisdorf, Rheinland, Germany, have invented certain new and useful Improvements in Ore-Briquetting, of which the following is a specification.

The object of this invention is to produce briquets of ore and slag which will not fall to pieces or crumble in transport to or exposure to the gases of the furnace in which the ore is to be smelted.

According to the present invention the pulverized charge, ore-dust, or fine-grained ore is caked with the aid of blast-furnace slag which has previously been treated in the presence of air, with or without admixtures. Tests have shown, that slag treated as set forth in the specification of my U. S. Patent No. 786,543 is best suited for the purpose indicated. However, the pulverization of the slag may also be performed by the direct action of a stream of air charged with pulverized admixtures, for example lime.

For the manufacture of ore-briquets for smelting purposes it has been proposed to mix pulverized iron ore and the like with ground blast-furnace slag, alumina and lime. The term "cement" cannot be accurately applied to the mass formed by these admixtures, though the said mass might be regarded as the raw material of cement, without the binding power imparted by burning. In practice it has been found that briquets made of the mixture described, or of similar mixtures, do not even possess sufficient durability to enable them to be conveyed to the blast furnace; or even if they can be placed whole in the blast-furnace the hot air-blast and the vapors and gases generated in the upper part of the furnace cause the cakes to crumble to dust, which is blown out of the furnace by the blast before it reaches the smelting zone, so that the iron is not obtained. It has also been proposed to treat solid slag with steam and then mix it with the ore without the addition of alumina and lime (U. S. Patent No. 833005). By this process the binding power of the slag is somewhat better developed but not sufficiently to prevent the crumbling of the briquets in the furnace before the smelting process has started.

In using ore briquets manufactured with blast-furnace slag which has been granulated in water, or has been exposed in a solid

state to the action of high pressure steam, it has been found that the minute cavities in the binding agent contain water which is evaporated when the briquets enter the upper zone of the smelting furnace, and the steam thus generated causes the briquets to crumble before they reach the smelting zone of the furnace.

In my present invention the binding agent is perfectly dry, and produces highly porous briquets, which are very permeable to gases, so that the reduction of the ore is materially assisted by the action of carbon monoxide. The improved briquets do not require a high degree of compression, such as would reduce their porosity, and the smaller proportion of binding agent required renders not only the manufacture of the briquets, but also the smelting process, more economical, and obviates the risk of loss of ore due to the embedding of ore-particles in a vitreous mass by which access of the reducing gases is prevented.

The pulverized slag is, according to the present invention, finely ground, either alone or with admixtures adapted to increase its binding power in case the said binding power is not naturally of a high order or has not previously been increased by means of admixtures introduced during the pulverizing process. The mealy powder obtained by the grinding process is intimately mixed with the ore, iron residue, ore-dust or the like and the mixture is molded under pressure in the usual manner. The cakes thus produced become in a comparatively short time sufficiently hard to be transported and subjected to the smelting process. This is due to the fact that during the pulverization of molten blast furnace slag the greater part of the sulfur contained therein is separated in the form of sulfur dioxide or sulfureted hydrogen, or both, so that the sulfur no longer counteracts the binding power of the cement. If admixtures are introduced during the pulverizing process the pulverization is accompanied by a process analogous to that which takes place in a cement furnace, and this process is considerably assisted by the burning of the sulfur and sulfureted hydrogen, so that the product is at least equivalent, in binding power, to Portland cement of good quality. It has, however, over Portland cement the important advantages that it reduces the cost of manufacturing the ore cakes, that smaller quantities thereof are suf-

ficient, that the cakes produced are more porous or permeable to the furnace gases, and that the chemical composition of the binding agent is better adapted for the purpose in view.

It has been found that the binding agent is considerably improved by adding a suitable quantity of alkaline salt, which may either be ground up with the slag or added after the grinding. By means of such addition the setting of the briquets is accelerated, and risk of cracking by frost is reduced, more particularly if the salt used is chlorid of calcium. On the other hand the presence of salts of the alkaline metals or earth metals prevents too rapid drying of the briquets, especially in summer, and enables artificial heat to be applied without risk of drying the mass before the briquets have set. Chlorid of calcium and chlorid of potassium also have the advantage that they assist in the elimination of sulfur, phosphorus, copper, zinc, arsenic and the like during the smelting process; by coaction with the silica in the slag and the iron oxid in the ore they cause, moreover, a fusing together of the briquet-particles and thus prevent sudden disintegration of the briquets by the heat of the smelting zone. Another advantage of the alkaline salts is that they render the slag basic and easily liquefiable, so that the proportion of lime can be increased without risk of producing a tough, viscous mass dangerous to the furnace. The alkalies also assist in the extraction of the manganese with the iron, which is an important advantage.

A very important advantage of using, for the manufacture of the ore briquets, slag which has been granulated in the presence of air, lies in the fact that the air-treatment of the slag renders it possible to use slags which are unsuitable for the briqueting processes hitherto used, by reason of the large proportion of manganese therein. Tests have been made with spiegel-eisen slag containing as much as 10% of manganese nearly free from phosphorus, with a high

proportion of lime, and it was found that by the dry granulation this slag is converted into a binding agent particularly suitable for briqueting, by reason of the large proportion of manganese. The manganese not only enriches the iron but also assists in eliminating sulfur. This latter function is important if the binding agent is used in conjunction with spent pyrites nearly free from phosphorus but containing a considerable proportion of sulfur. If the presence of manganese in the iron is not desired, a considerable proportion of manganese in the binding agent is still useful for rendering the slag basic and easily liquefiable and for binding the sulfur present.

What I claim as my invention and desire to secure by Letters Patent of the United States is:—

1. In ore briqueting the process of producing slag cement which consists in granulating blast furnace slag in the presence of air, grinding the product in the presence of materials adapted to strengthen the cementitious properties mixing the product with ore and forming same into briquets.

2. In ore briqueting, the process of producing slag cement which consists in granulating blast furnace slag in the presence of air, carrying in the form of dust material adapted to strengthen the cementitious properties of the slag, grinding the product mixing the same with ore and forming same into briquets.

3. In ore briqueting the process of producing slag cement which consists in granulating blast furnace slag in the presence of air, grinding the product in the presence of alkaline salts adapted to strengthen the cementitious properties mixing the product with ore and forming same into briquets.

In witness whereof I have signed this specification in the presence of two witnesses.

WILHELM LESSING.

Witnesses:

LOUIS VANDORN,  
H. STELZER.